

June 24, 1930.

L. D. KAY

1,768,362

PROCESS OF MAKING GRILLE WORK

Filed May 23, 1928



Inventor

Lloyd D. Kay;

*Lloyd D. Kay*

By

Attorneys

## UNITED STATES PATENT OFFICE

LLOYD D. KAY, OF LOS ANGELES, CALIFORNIA, ASSIGNOR TO KAY-BRUNNER STEEL PRODUCTS INC., OF LOS ANGELES, CALIFORNIA, A CORPORATION OF DELAWARE

## PROCESS OF MAKING GRILLE WORK

Application filed May 23, 1928. Serial No. 279,910.

This invention relates to ornamental grille work which is used largely in the construction of ornamental gates, "cages" in banks, and ornamental iron work such as used in building construction. This grille work is very popular but has heretofore been generally constructed entirely by hand and is consequently very expensive.

The general object of this invention is to provide a simple process for constructing grille work which will enable the grille work to be produced at a relatively low cost but which will have the strength and substantially the same appearance as ordinary grille work.

Further objects of the invention will appear hereinafter.

The invention consists in the novel steps and combination of steps to be described hereinafter, all of which contribute to produce an efficient process of making grille work. The invention consists also in the grille work resulting from the process.

A preferred embodiment of the invention is described in the following specification, while the broad scope of the invention is pointed out in the appended claims.

In the drawing:

Figure 1 is a vertical section through a balustrade having grille work ends embodying my invention.

Figure 2 is a detail showing a portion of the end of the balustrade broken away.

In practicing the invention, I provide a frame 1 which is preferably constructed of wrought iron or steel. This frame may have any shape adapting it to the particular purpose for which the grille work is to be employed. In the present instance this frame would constitute the framework of a balustrade and is constructed with vertical frame members 2 which are secured against the face of a wall 3. The frame includes also two horizontal foot bars 4 which extend longitudinally of the balustrade and may include hand rails 5 and 6 which extend horizontally at the ends of the construction and connect at their outer ends to longitudinal rails 7 and 8. The rails 7 and 8 may be supported on ornamental corner

posts or stanchions 9. If desired the stanchions may be provided with ornamental caps such as the cap 10.

After constructing the frame by welding these parts together or otherwise connecting them, I employ ornamental castings such as the castings 11 and 12. In the present instance the latter casting is of suitable form and dimensions to enable it to be set between the horizontal rails 5 and 6 so that the casting touches these rails at contact points 13, and at one end touches the vertical frame member 2 at a contact point 14. The outer end of the casting touches the corner post 9 at a contact point 15. This casting may be formed of two ornamental scrolls connected by an inclined bar. It may have any desired shape.

The space between the foot bars 4 and the rail 6 is filled by an ornamental casting 11 which is set in place, and this casting 11 is of sufficient dimension and proper form to touch the rails 4 and 6 at the contact points 16. It also preferably touches the frame member 2 at a plurality of points such as points 17. At its outer portion the ornamental casting 11 touches the stanchion 9 at a plurality of points 18.

If desired, under the balustrade an ornamental bracket casting 19 may be provided which touches the under sides of the rails 4 at several points 20 and this bracket also touches the frame member 2 at the point 21.

After setting the castings in contact with the frame, I then weld all the points of contact to produce welded joints such as indicated by the dotted lines 22 at these points.

In order to facilitate the making of these welded joints, I prefer to employ wrought iron or steel having a known carbon content. The frame members are preferably made of rolled iron or steel and preferably have a carbon content of about one-tenth of one percent. The castings should have a carbon content conforming substantially to this but the carbon content in the castings may run as high as about twenty-five-hundredths of one percent. The carbon content in the

frame may run as high as about fifteen-hundredths of one percent.

As is well known, castings are relatively hard and brittle. Castings of irregular form such as illustrated and such as are used in ornamental iron work may vary considerably in their dimensions and hence in setting the castings in the frame it may be necessary to force the castings somewhat out of their natural form. This may set up dangerous strains in the castings. In order to soften the castings and prepare them for receiving hammer blows, I anneal the structure after the joints have all been welded. This annealing may be made through a wide range of temperature. Any temperature from about 650° F. to 1650° F. will be found satisfactory. After annealing the structure, I hammer the castings and the frame with a small hammer. These blows assist in eliminating the internal stresses in the castings, and the softened condition of the castings due to the annealing prevents any possibility of their being cracked by the blows. The softened surface of the castings enables the hammer to indent the surface of the castings as indicated in the detail (Figure 2).

In this way ornamental iron work can be produced at a relatively low cost. The castings can be very inexpensively produced and may have a high degree of ornamentation. In this way very pleasing ornamental iron work can be produced which closely resembles ordinary grille work constructed entirely of wrought iron beaten and bent into the desired shape.

It will be evident that in welding the contact points, it is only necessary to weld a sufficient number of them to securely hold the cast portions in place.

It is understood that the embodiment of the invention described herein is only one of the many embodiments this invention may take, and I do not wish to be limited in the practice of the invention, nor in the claims, to the particular embodiment set forth.

What I claim is:

1. A process of constructing grille-work which consists in constructing a frame of wrought iron or steel, setting castings of ornamental form in contact with the frame, welding the castings to the frame at the points of contact, and annealing the structure thereafter.

2. A process of making grille-work which consists in constructing a frame of wrought iron or steel, setting ornamental castings in the frame having contact points touching the frame, welding the castings to the frame at such contact points, annealing the structure thereafter to soften the material of the castings, and then hammering the castings to reduce their internal stresses.

3. A process of making grille-work which

consists in constructing a frame of wrought iron or steel having a known carbon content, setting ornamental castings in the frame having known carbon content conforming to the carbon content of the material of the frame and so that the castings touch the frame at contact points, welding the castings to the frame at such contact points, and annealing the structure thereafter to soften the material of the castings.

4. A process of making grille-work which consists in constructing a frame of wrought iron or steel having a carbon content of approximately one-tenth of one per cent, setting ornamental castings in the frame having a carbon content of approximately two-tenths of one per cent, and so that the castings touch the frame at contact points, welding the castings to the frame at such contact points, annealing the structure thereafter to soften the material of the castings, and then hammering the castings to reduce their internal stresses.

5. A process of making grille-work which consists in constructing a frame of wrought iron or steel having a carbon content of approximately one-tenth of one per cent, setting ornamental castings in the frame having a carbon content of approximately two-tenths of one per cent, and so that the castings touch the frame at contact points, welding the castings to the frame at such contact points, annealing the structure thereafter to soften the material of the castings, hammering the surface of the frame to ornament the same, and then hammering the surface of the castings to reduce their internal stresses and to increase their ornamental appearance.

6. A process of making grille-work which consists in constructing a frame of wrought iron or steel having a carbon content of approximately one-tenth of one per cent, setting castings in the frame having a carbon content of approximately two-tenths of one per cent, and so that the castings touch the frame at contact points, welding the castings to the frame at such contact points, annealing the structure thereafter to soften the material of the castings, and hammering the surface of the castings to reduce their internal stresses and enhance their ornamental appearance, and also hammering the surface of the frame.

Signed at Los Angeles, California, this 3rd day of May, 1928.

LLOYD D. KAY.